

# UNITED STATES PATENT OFFICE.

WILBUR ALSON HENDRYX, OF DENVER, COLORADO.

## METHOD OF TREATING SULFID ORES.

No. 893,580.

Specification of Letters Patent.

Patented July 14, 1908.

Application filed November 20, 1906. Serial No. 344,321.

To all whom it may concern:

Be it known that I, WILBUR ALSON HENDRYX, a citizen of the United States, residing at Hotel Metropole, in the city of Denver, in the county of Denver and State of Colorado, have invented new and useful Improvements in Methods of Treating Sulfid Ores, of which the following is a specification.

This invention is a method of treating ores, and more particularly ores containing sulfid of copper, the object of the invention being to provide a method whereby metals such as copper may be extracted directly from their sulfid ores and recovered as a reguline deposit.

In treating pyritic ores containing sulfid of copper together with some sulfid of iron I prefer to proceed as follows: The suitably ground ore is mixed in a vessel provided with a mechanical agitator with dilute sulfuric acid, the sulfuric acid being added in approximately the theoretical proportion required to dissolve the copper of the ore, or in some excess of such proportion. The solution is preferably heated to about 120-160 degrees Fahrenheit. Insoluble anodes, preferably of lead, and cathodes which may also be of lead or of copper are suitably disposed in the solution, and a suitable electric current is transmitted throughout the operation. For this purpose I prefer to employ apparatus substantially as described in my prior patent No. 785,214, granted March 21, 1905, the parts of the same being constructed of suitable materials to withstand the solutions employed.

Under the conditions described the copper sulfid is not directly dissolved by the sulfuric acid, but sulfid of iron is dissolved, yielding ferrous sulfate which in the region of the insoluble anodes is converted into ferric sulfate. This salt attacks the copper sulfid, converting it into copper sulfate, and is itself reduced to ferrous sulfate, but is immediately reoxidized to ferric sulfate at the anodes and in presence of the ore. In this manner a complete and rapid solution of the copper sulfid is effected. Meantime a coherent deposit of copper is formed upon the cathodes, although under the most economical working conditions the whole of the copper is not deposited. So long as sufficient copper is present in solution and is being deposited therefrom, there is little or no tendency to the reduction of the iron salts at the cathodes, and the solution of the sulfid and the regenera-

tion of the solvent ferric salts is rapid. After the solution of the copper is complete the pulp is discharged into a sand or other filter, and the clear solution therefrom is passed through one or more electrolytic cells provided with anodes of lead and cathodes of copper, lead or the like. In these cells further portions of copper are deposited and any iron which may be present in the ferrous state is oxidized. Preferably the solution should not be so far depleted of copper in these cells as to render it difficult to secure a reguline deposit of the metal or to subject the ferric salts to reduction by hydrogen liberated at the cathodes.

The solution flowing from the electrolytic cells and containing in addition to some copper the fully regenerated solvent is employed for the treatment of fresh batches of ore.

While I have described the employment of sulfuric acid my invention is not restricted thereto, as it will be obvious that the solvent initially added may be another acid, as hydrochloric acid, or other solvent for copper sulfid or a body capable of giving rise to such solvent, as for instance ferric or ferrous salts. In case hydrochloric acid or a chlorid is employed the anode will preferably be of graphite.

The precipitating cells for the copper may be of any usual type, and are preferably provided with a large electrode surface, whereby the metal is rapidly deposited and any ferrous salts are quickly oxidized. To this end they preferably comprise vats or troughs containing a large number of electrodes so disposed that the solution in continuous flow encounters anodes and cathodes repeatedly and in alternation.

I claim:

1. The method of treating ores containing copper which consists in reacting upon the same with a solution containing a ferric salt and simultaneously separating copper by electrolysis with insoluble anodes, thereby regenerating the ferric salt in presence of the ore.

2. The method of treating ores containing copper which consists in reacting upon the same with a solution containing ferric sulfate and simultaneously separating copper by electrolysis with insoluble anodes, thereby regenerating the ferric sulfate in presence of the ore.

3. The method of treating ores containing copper which consists in reacting upon the

same with a solution containing a ferric salt and simultaneously separating the copper by electrolysis with insoluble anodes, thereby regenerating the ferric salt in presence of the ore, separating the solution and electrodepositing copper therefrom.

4. The method of treating ores containing copper which consists in reacting upon the same with a solution containing a ferric salt and simultaneously separating copper by electrolysis with insoluble anodes, thereby regenerating the ferric salt in presence of the ore, separating the solution and electrodepositing copper therefrom by passing the solution successively in contact with suitable cathodes and insoluble anodes.

5. The method of treating ores containing copper which consists in reacting upon the same with a solution containing a ferric salt and simultaneously separating copper by electrolysis with insoluble anodes, thereby regenerating the ferric salt in presence of the ore, separating the resulting solution, electro-

depositing copper therefrom by passing it alternately and repeatedly in contact with insoluble anodes and suitable cathodes, and subjecting additional quantities of ore to the solvent action of the solution.

6. The method of treating ores containing copper and iron which consists in reacting upon the same with an acid and simultaneously separating copper by electrolysis with insoluble anodes, thereby regenerating the solvent liquor in presence of the ore.

7. The method of treating ores containing copper and iron which consists in reacting upon the same with sulfuric acid and simultaneously separating copper by electrolysis with insoluble anodes, thereby regenerating the solvent liquor in presence of the ore.

In testimony whereof I affix my signature in presence of two witnesses.

WILBUR ALSON HENDRYX.

Witnesses:

THEODORA WELLS,  
CHAS. R. DAVIES.